

G. H. HARDMAN.

COATING FOR RAILROAD TIES AND METHOD OF APPLYING THE SAME.

APPLICATION FILED APR. 5, 1922.

1,418,708.

Patented June 6, 1922.



Fig. 1



Fig. 2

INVENTOR.  
George H. Hardman  
BY  
Horatio S. Bellows  
ATTORNEY

# UNITED STATES PATENT OFFICE.

GEORGE H. HARDMAN, OF FALL RIVER, MASSACHUSETTS.

## COATING FOR RAILROAD TIES AND METHOD OF APPLYING THE SAME.

1,418,708.

Specification of Letters Patent. Patented June 6, 1922.

Application filed April 5, 1922. Serial No. 549,919.

To all whom it may concern:

Be it known that I, GEORGE H. HARDMAN, a citizen of the United States, residing at Fall River, in the county of Bristol and State of Massachusetts, have invented certain new and useful Improvements in Coatings for Railroad Ties and Methods of Applying the Same, of which the following is a specification.

10 My invention relates to rail-road ties and more particularly to those constructed of wood.

The essential objects of my invention are the preservation of the tie against heat, cold, moisture, and climatic conditions whereby its period of utility is prolonged, and to attain this end by a simple and inexpensive means.

To the above ends essentially my invention consists in such parts and in such combinations of parts, and in such steps and succession of steps as fall within the scope of the appended claims.

In the accompanying drawings which 25 form a part of this specification,

Figure 1 is a perspective view of a rail-road tie embodying my invention, and

Figure 2, a transverse section of the same.

30 Like reference characters indicate like parts throughout the views.

In the drawings 5 represents the body of a wooden railroad tie which may be of any usual preferred construction either solid or 35 sectional. In the form thereof herein shown the body is sectional comprising longitudinally disposed strips 7 through which pass transversely at intervals bolts or tie rods 10 provided with bifurcated ends forming 40 straps or fingers 12 embracing the body seated in peripheral grooves 13 therein.

Enclosing the exterior of the body is a

covering of asphalt and asbestos. The method of applying the covering herein shown consists in surrounding the body 45 with a film or thin layer 15 of a preservative such as asphalt. This may be done by dipping the body 5 into hot liquid asphalt. Next a film or thin layer 17 of asbestos is applied by rolling the asphalt covered body 50 in a mass of pulverized asbestos while the asphalt is still hot and soft, or by blowing the asbestos upon the same while in the described condition; or by rubbing the asbestos into the asphalt. 55

For the purpose of illustration the thickness of each of the films or layers 15 and 17 are herein shown greatly exaggerated.

The asbestos coating prevents the cracking of the asphalt by cold or the melting of 60 the same by heat which would otherwise occur.

I claim:

1. In a rail-road tie, the combination of the body and a coating of asphalt and asbestos enclosing the body. 65

2. In a rail-road tie, the combination of the body, and a coating comprising a layer of asphalt surrounding the body, and a layer of asbestos superposed on the layer 70 of asphalt.

3. The method of preserving wooden railroad ties consisting in covering the tie with a coating of hot asphalt, and next applying a coating of asbestos to the first coating 75 while the asphalt is in an unhardened state.

4. The method of preserving wooden railroad ties consisting in covering the tie with an adhesive coating, and next applying a coating of asbestos to the first coating. 80

In testimony whereof I have affixed my signature.

GEORGE H. HARDMAN.